

## UNITED STATES PATENT OFFICE

THOMAS H. ROGERS, OF HAMMOND, INDIANA, ASSIGNOR TO STANDARD OIL COMPANY,  
OF WHITING, INDIANA, A CORPORATION OF INDIANA

## COLORED WAX AND CANDLE

No Drawing.

Application filed August 9, 1928. Serial No. 298,626.

This invention relates to colored waxes and candles. Such candles may be composed of colored wax or may have a coating of colored wax applied thereto by dipping or in 5 other suitable manner.

Considerable difficulty has been experienced with such candles due to the fading of the dyes with which the wax is colored. This difficulty is particularly experienced with 10 pink, lavender and red shades in waxes which contain rhodamine B and to a lesser extent with waxes dyed with Chinoline yellow. This fading occurs not only when the candles are exposed to strong light, but also 15 while they are stored in the dark.

I have now discovered that this difficulty may be practically completely avoided by adding minute quantities of certain substances to the dyed wax. Thus I have found 20 that minute quantities, for example, substantially less than 1% of beta naphthol when added to the colored wax, reduce the fading practically to zero.

For example, the most troublesome color 25 with which I am acquainted is a "shell pink", which is generally applied by dipping white candles in a coating composition comprising approximately equal parts of paraffine wax and stearic acid with rhodamine B to color. 30 A candle thus colored when stored in the dark at a temperature of 100° F., will become practically colorless within two weeks. The addition of 0.025% of beta naphthol to the colored wax stabilizes the color so that 35 it shows only very slight fading after six weeks at the same temperature. At room temperature, an unstabilized candle of this color will show fading in about a month, while stabilized candles show no fading after 40 about five months.

Not only has the added beta naphthol a 45 very valuable result in the finished product, but it exercises valuable effects during the manufacturing operation. Thus in the course of dipping, during which a bath of

colored wax is maintained at a temperature around 150° F., there is appreciable fading which is reduced enormously when the wax contains beta naphthol.

Instead of beta naphthol, I may employ 50 other substances having the properties of beta naphthol. For example I may employ elemental sulfur in finely divided form. Such sulfur may be incorporated in the wax to the extent of around 0.1%, and in that 55 proportion exerts a highly efficient color stabilizing effect.

I claim:

1. The method of preventing fading of dye in dyed wax which fades on standing which consists in adding to said wax approximately 0.025% of beta naphthol.
2. A dyed wax comprising paraffin wax, stearic acid, a dye stuff and about 0.025% of beta naphthol.
3. A dyed wax of a character normally fading on standing and containing less than 1% of beta naphthol, whereby fading is prevented.
4. The method of preventing fading of the dye in colored wax mixtures comprising paraffin wax and stearic acid, which comprises adding to such dyed mixture less than 1% of beta-naphthol.
5. The method of preventing fading of 75 dye-colored waxes which normally fade on standing, which consists in adding to such waxes less than 1% of beta-naphthol.
6. The method of preventing fading of 80 rhodamine-B and Chinoline yellow when used in coloring petroleum waxes which fade on standing, which consists in adding to said waxes a small proportion of beta naphthol less than one percent.

85

THOMAS H. ROGERS.

90